



US007258177B2

(12) **United States Patent**  
**Liang et al.**

(10) **Patent No.:** **US 7,258,177 B2**  
(45) **Date of Patent:** **\*Aug. 21, 2007**

(54) **FRACTURE AND WEAR RESISTANT COMPOUNDS AND ROCK BITS**

(75) Inventors: **Dah-Ben Liang**, Woodlands, TX (US); **Anthony Griffio**, The Woodlands, TX (US)

(73) Assignee: **Smith International, Inc.**, Houston, TX (US)

(\*) Notice: Subject to any disclaimer, the term of this patent is extended or adjusted under 35 U.S.C. 154(b) by 0 days.

This patent is subject to a terminal disclaimer.

(21) Appl. No.: **11/415,657**

(22) Filed: **May 2, 2006**

(65) **Prior Publication Data**

US 2006/0254828 A1 Nov. 16, 2006

**Related U.S. Application Data**

(63) Continuation of application No. 10/396,261, filed on Mar. 25, 2003, now Pat. No. 7,036,614, which is a continuation-in-part of application No. 10/017,404, filed on Dec. 14, 2001, now Pat. No. 6,655,478.

(51) **Int. Cl.**  
**E21B 10/36** (2006.01)  
(52) **U.S. Cl.** ..... **175/374; 175/425; 175/428**  
(58) **Field of Classification Search** ..... **175/374, 175/425, 428**  
See application file for complete search history.

(56) **References Cited**

**U.S. PATENT DOCUMENTS**

7,036,614 B2 \* 5/2006 Liang et al. ..... 175/374  
7,048,080 B2 \* 5/2006 Griffio et al. ..... 175/375  
2004/0140133 A1 \* 7/2004 Liang ..... 175/428

\* cited by examiner

*Primary Examiner*—William Neuder

(74) *Attorney, Agent, or Firm*—Osha Liang LLP

(57) **ABSTRACT**

An insert for a rock bit that includes tungsten carbide particles, and a cobalt binder disposed around the particles, wherein a grain size of the tungsten carbide particles and a content of the cobalt binder are selected to provide a fracture toughness of at least about 18 ksi (in)<sup>0.5</sup>, a wear number of at least about 2, and a hardness of 85 to 87 Ra is disclosed.

**15 Claims, 9 Drawing Sheets**



**FIG. 1**



FIG. 2



FIG. 3A



FIG. 3B



FIG. 4A



FIG. 4B

## COARSE GRAIN CARBIDE GRADES &amp; HARDNESS SPEC

| GRADE | NOMINAL HARDNESS (RA) | GRADE | NOMINAL HARDNESS (RA) | GRADE | NOMINAL HARDNESS (RA) |
|-------|-----------------------|-------|-----------------------|-------|-----------------------|
|       |                       | 916   | 83.8                  |       |                       |
|       |                       | 914   | 84.4                  |       |                       |
| 1012  | 84.4                  | 912   | 85.0                  | 812   | 85.6                  |
| 1010  | 85.0                  | 910   | 85.6                  | 810   | 86.2                  |
| 1008  | 85.6                  | 908   | 86.2                  | 808   | 86.8                  |

*FIG. 5*



FIG. 6



FIG. 7

## FRACTURE AND WEAR RESISTANT COMPOUNDS AND ROCK BITS

### CROSS-REFERENCE TO RELATED APPLICATIONS

This application claims the benefit under 35 U.S.C. § 120 as a continuation of U.S. patent application Ser. No. 10/396,261, filed Mar. 25, 2003, now U.S. Pat. No. 7,036,614, which is a continuation-in-part of U.S. application Ser. No. 10/017,404, filed Dec. 14, 2001, now U.S. Pat. No. 6,655,478, which are incorporated by reference in their entirety.

### BACKGROUND OF INVENTION

#### 1. Field of the Invention

The invention relates generally to fracture and wear resistant rock bits. More specifically, the invention relates to compositions for inserts used on rock bits which enhance the useful life of the bit.

#### 2. Background Art

Drill bits used to drill wellbores through earth formations generally are made within one of two broad categories of bit structures. Drill bits in the first category are generally known as "fixed cutter" or "drag" bits, which usually include a bit body formed from steel or another high strength material and a plurality of cutting elements disposed at selected positions about the bit body. The cutting elements may be formed from any one or combination of hard or superhard materials, including, for example, natural or synthetic diamond, boron nitride, and tungsten carbide.

Drill bits of the second category are typically referred to as "roller cone" bits, which include a bit body having one or more roller cones rotatably mounted to the bit body. The bit body is typically formed from steel or another high strength material. The roller cones are also typically formed from steel or other high strength material and include a plurality of cutting elements disposed at selected positions about the cones. The cutting elements may be formed from the same base material as is the cone. These bits are typically referred to as "milled tooth" bits. Other roller cone bits include "insert" cutting elements that are press (interference) fit into holes formed and/or machined into the roller cones. The inserts may be formed from, for example, tungsten carbide, natural or synthetic diamond, boron nitride, or any one or combination of hard or superhard materials.

Breakage or wear of the inserts, among other factors, limits the longevity of a drill bit. Inserts used with a rock bit are generally subjected to high wear loads from contact with a borehole wall, as well as high stresses due to bending and impact loads from contact with a borehole bottom. The high wear loads can also cause thermal fatigue in the inserts, which initiates surface cracks on the inserts. These cracks are further propagated by a mechanical fatigue mechanism that is caused by the cyclical bending stresses and/or impact loads applied to the inserts. Fatigue cracks may result in chipping, breakage and failure of inserts.

Inserts that cut the corner of a borehole bottom, such as gage inserts are subject to a significant amount of thermal fatigue. Thermal fatigue is caused by heat generated on the gage side of an insert by friction when the insert engages the borehole wall and slides into a bottom-most crushing position. When the insert rotates away from the bottom, it is quickly cooled by the surrounding circulating fluid. Repetitive heating and cooling of the insert initiates cracking on the outer surface of the insert. Thermal fatigue cracks then propagate through the body of the insert when the crest of

the insert contacts the borehole bottom (because of the high contact stresses). The time required to progress from heat checking, to chipping, and eventually to broken inserts depends upon formation type, rotational speed of their bit, and applied weight on bit, among other factors.

The interior rows are also subject to thermal fatigue caused by scraping the borehole bottom. The amount of scraping varies from row to row and is influenced by bit offset and cone to bit speed ratio.

Cemented tungsten carbide generally refers to tungsten carbide (WC) particles dispersed in a binder metal matrix, such as iron, nickel, or cobalt. Tungsten carbide in a cobalt matrix is the most common form of cemented tungsten carbide, which is further classified by grades based on the grain size of WC and the cobalt content.

Tungsten carbide grades are primarily made in consideration of two factors that influence the lifetime of a tungsten carbide insert: wear resistance and toughness. As a result, inserts known in the art are generally formed of cemented tungsten carbide with average grain sizes about less than 3  $\mu\text{m}$  as measured by ASTM E-112 method, cobalt contents in the range of about 6-16% by weight and hardness in the range of about 86 Ra to 91 Ra.

For a WC/Co system, it is typically observed that the wear resistance increases as the grain size of tungsten carbide or the cobalt content decreases. On the other hand, the fracture toughness increases with larger grains of tungsten carbide and greater percentages of cobalt. Thus, fracture toughness and wear resistance (i.e., hardness) tend to be inversely related: as the grain size or the cobalt content is decreased to improve the wear resistance of a specimen, its fracture toughness will decrease, and vice versa.

Due to this inverse relationship between fracture toughness and wear resistance (i.e., hardness), the grain size of tungsten carbide and the cobalt content are selected to obtain desired wear resistance and toughness. For example, a higher cobalt content and larger WC grains are used when a higher toughness is required, whereas a lower cobalt content and smaller WC grains are used when a better wear resistance is desired.

### SUMMARY OF INVENTION

In one aspect, the present invention relates to a fracture and wear resistant rock bit, which includes a bit body, and at least one roller cone rotatably mounted on the bit body adapted such that at least one row of cutting elements disposed on the at least one roller cone defines a row. At least one cutting element disposed on the gage or inner row has a fracture toughness of at least 18 ksi  $(\text{in})^{0.5}$  and a wear number of at least 2.0.

In one aspect, the present invention relates to an insert for a rock bit that includes tungsten carbide particles, and a cobalt binder disposed around the particles, wherein a grain size of the tungsten carbide particles and a content of the cobalt binder are selected to provide a fracture toughness of at least about 18 ksi  $(\text{in})^{0.5}$  and a wear number of at least about 2.

Other aspects and advantages of the invention will be apparent from the following description and the appended claims.

### BRIEF DESCRIPTION OF DRAWINGS

FIG. 1 shows a perspective view of an roller cone drill bit made in accordance with an embodiment of the invention.

FIG. 2 shows a cross-sectional view of a roller cone in accordance with an embodiment of the invention.

FIGS. 3a and 3b show exemplary grain size distributions for compositions “510” and “616,” respectively.

FIGS. 4a and 4b show exemplary grain size distributions for compositions “916” and “812,” respectively.

FIG. 5 is a table listing assigned grade size and hardness.

FIG. 6 shows a graphical comparison of normalized fatigue resistance index for conventional carbide bits and carbide bits in accordance with embodiments of the present invention.

FIG. 7 shows a graphical comparison of fracture toughness vs. wear resistance for conventional carbide bits and carbide bits in accordance with embodiments of the present invention.

#### DETAILED DESCRIPTION

It has been determined that when drilling certain formations (for example, carbonate formations), inserts having a high fracture toughness with adequate wear resistance and low hardness exhibit improved performance and/or longevity when compared to conventional inserts. This can be accomplished by using coarse grain carbide grades.

FIG. 1 shows a typical roller cone bit used for drilling boreholes in earth formations. The drill bit 10 comprises a bit body 20 and threads 14 formed at an upper end and three legs 22 formed at a lower end. The threads 14 are adapted to couple the bit 10 to a drillstring or bottom hole assembly (BHA) (not shown) used to drill a wellbore (not shown).

Each of three roller cones 16 is rotatably mounted on a corresponding leg 22 proximate the lower end of the bit body 20. A plurality of cutting elements, which in this case comprise inserts 18 that are typically formed from cemented tungsten carbide, are press-fit (or interference fit), brazed, or otherwise affixed in holes (not shown separately in FIG. 1) formed in the roller cones 16. Lubricant for the roller cones 16 is provided to the journals (19 in FIG. 2) on which the roller cones 16 are rotatably mounted from grease reservoirs 24 in the bit body 20. This configuration is generally used for sealed-bearing rock bits. For open-bearing (unsealed) rock bits, such as those typically used in mining applications, there typically are no grease reservoirs.

Referring to FIG. 2, when in use, the drill bit 10 is threaded onto a lower end of the drillstring (not shown) and lowered into a wellbore or borehole. The drillstring is rotated by, for example, a rig rotary table (not shown) or a top drive (not shown), and the inserts 18 in the cones 16 engage the bottom and side of the borehole 25. As the bit rotates, the cones 16 rotate on the bearing journals 19 and drill the borehole 25. Weight on bit (WOB) is applied to the drillstring and to the formation by the inserts 18, and the formation is generally crushed and chipped (or scraped) by the inserts 18. A drilling fluid (often referred to as “drilling mud”) is usually pumped through the drillstring to the drill bit (10 in FIG. 1) and is ejected through nozzles (26 in FIG. 1) disposed in the bit body (20 in FIG. 1). The drilling fluid then travels up a borehole annulus (not shown) formed between the exterior of the drillstring and the borehole 25 wall. The drilling fluid transports most of the formation cuttings drilled by the bit to the surface. In addition, the drilling fluid serves to cool and clean the inserts 18 and roller cones 16 as the borehole 25 is being drilled.

FIG. 2 also shows a lower portion of the leg 22 that supports a journal bearing 19. A plurality of cone retention balls 21 (e.g., “locking balls”) and roller bearings 12a and 12b surround the journal 19. An O-ring 28, located within in

an O-ring groove 23, seals the bearing assembly. The type of seal and roller cone retention device are only shown here to illustrate the general structure of a roller cone drill bit and are not intended to limit the invention.

The cones 16 include multiple rows of the inserts 18, and the roller cones 16 generally include a heel portion 17 located between gage row inserts 15 and the O-ring groove 23. A plurality of heel row inserts 30 are approximately equally spaced about a circumference of the heel 17. The heel row inserts 30 and the gage row inserts 15 act together to drill a gage diameter of the borehole 25. The interior row inserts 18 are generally arranged in, for example, concentric rows, and they serve to crush and chip the earth formations being drilled. Although the geometric shape of the inserts is not critical, it is preferred that they have a semi-round top, a conical top, or a chiseled top.

In one embodiment according to the present invention, at least inner row insert 18 disposed on the bit 10 comprises a tungsten carbide insert, having a coarse (large) grain size, i.e., an average grain size larger than approximately 4  $\mu\text{m}$  as determined by the ASTM E-112 method. Preferably, the insert has a fracture toughness of at least 18 ksi  $(\text{in})^{0.5}$  when measured by the ASTM B-771 method. Additionally, the insert has a wear number of at least 2.0 when measured by the ASTM B-611 method. More preferably, the insert also has a hardness range of about 85.0 to about 87.0 Rockwell “A” hardness (Ra). In order to achieve the above fracture toughness and wear resistance, the cobalt content and the grain size of the carbide should be carefully selected.

Currently, conventional inserts having a hardness between 85 and 87 Ra are used for interior row application, i.e. grade 614, 616, etc. Typical prior art bits use inserts within this hardness range having toughness below 17 or between 15 and 17 ksi  $(\text{in})^{0.5}$  and wear numbers between 1.8 to 2.5 for most inner row applications. Gage row inserts of the bits normally have a higher wear number than the interior row inserts. It was believed that gage inserts needed the wear resistance, because of the large amount of borehole wall contact encountered. Accordingly, toughness was sacrificed to gain wear resistance. However, when drilling some soft formation such as carbonates, the wear resistance of the inserts is not a major concern because the rocks are not very abrasive. Carbide grades formed in accordance with embodiments of the present invention, however, provide insert toughness and an ability to resist breakage after thermal fatigue cracks have formed.

Embodiments of the present invention, having a hardness range from about 85 to 87 Ra are particularly suitable for inner row drilling in more abrasive formations.

In general, embodiments of the invention relate to inserts having a defined cobalt content and an average carbide particle size. Because tungsten carbide disposed in a cobalt matrix is representative of wear-resistant material, embodiments of the invention are explained with reference to a WC/Co system. However, it should be understood that embodiments of the invention are not limited to a WC/Co system. Specifically, transition metal borides, transition metal carbides, transition metal nitrides, and other transition metal carbides are specifically within the scope of the present invention.

The following naming convention is used to describe embodiments of the invention. According to this convention, carbide inserts are given a three (or four) digit code name, where the first digit indicates the relative particle size of tungsten carbides and the latter two digits indicate the cobalt content. For example, “616” represents an insert having a carbide relative particle size of 6 and a 16% cobalt

content by weight. Note that the "relative" particles sizes used in this naming convention do not indicate actual particle sizes. The average carbide particle size for **616**, as measured by the ASTM E-112 method, is approximately 2.8 um.

In one embodiment, fracture toughness and wear resistance of an insert having a cobalt content of about 12% and a carbide relative particle size of about 8 were determined. The average carbide particle size as measured by ASTM E-112 method is approximately 4.9 um. This composition, termed "**812**", exhibited a fracture toughness of about 18 ksi (in)<sup>0.5</sup> (as measured in accordance with the ASTM B-771 method) and a wear number of about 2.2 (as measured in accordance with the ASTM B-611 method).

In another embodiment, fracture toughness and wear resistance of an insert having a cobalt content of about 12% and a carbide relative particle size of about 9 were determined. The average carbide particle size as measured by ASTM E-112 method is approximately 5.8 um. This composition, termed "**912**", exhibited a fracture toughness of about 20 ksi (in)<sup>0.5</sup> (as measured in accordance with the ASTM B-771 method) and a wear number of about 2.2 (as measured in accordance with the ASTM B-611 method).

In another embodiment, fracture toughness and wear resistance of an insert having a cobalt content of about 14% and a carbide particle size number of about 9 were determined. The average carbide particle size as measured by ASTM E-112 method is approximately 5.8 um. This composition, termed "**914**", exhibited a fracture toughness of about 21 ksi (in)<sup>0.5</sup> (as measured in accordance with the ASTM B-771 method) and a wear number of about 1.8 (as measured in accordance with the ASTM B-611 method).

In another embodiment, fracture toughness and wear resistance of an insert having a cobalt content of about 16% and a carbide particle size number of about 9 were determined. The average carbide particle size as measured by ASTM E-112 method is approximately 5.8 um. This composition, termed "**916**", exhibited a fracture toughness of about 22 ksi (in)<sup>0.5</sup> (as measured by the ASTM B-771 method) and a wear number of about 1.6 (as measured by ASTM B-611).

These results were then compared against conventional carbide inserts, which generally use carbides having a relative particle size number of about 3 to about 6 and cobalt content of about 6% to about 16% by weight. The average carbide particle size as measured by the ASTM E-112 method is approximately less than 3.0 um for above conventional carbide inserts.

FIGS. 3a, 3b, 4a, and 4b show exemplary grain size distributions for compositions "**510**," "**616**," "**916**," and "**812**," respectively. As the Figures show, all of the compositions have a distribution of grain sizes. The average grain size is listed under the heading "average" in the Figures.

The above embodiments reference particular particle sizes in determining what "grade" to assign a given composition. However, in practice, this is difficult because of the number of particles within a given sample. Particles within a given sample tend to be non-uniform, so the values given above represent a "best estimate" approach to assigning the grade of carbide (i.e., assigning the first number in the three or four number composition code).

FIG. 5 shows an alternative method of assigning the grades. As the average carbide particle increases in size, the "nominal hardness" of the compound decreases. The hardness of a composition may be relatively easily tested, by a variety of known methods. Within the present invention, grades are assigned based on increments of 0.6 Ra. That is,

for a given amount of cobalt (e.g., 12%), as the relative grade size increases from 8 to 10, the nominal hardness drops from 85.6 (for "**812**") to 85.0 (for "**912**") to 84.4 ("**1012**"). It should also be noted that as the amount of cobalt is increased (which is a ductile material) by 2%, the nominal hardness reduces by approximately the same amount. Thus, as the amount of cobalt within a given tungsten carbide grade is increased, the nominal hardness decreases.

FIG. 6 shows a comparison of normalized thermal fatigue resistance index between conventional carbide inserts (indicated by the composition numbers **616**, **614**, and **510**) and the coarse grain carbide of the present invention (indicated by the composition numbers **916**, **914**, **912**, **814**, **712**, and **812**). In FIG. 6, the coarse grain carbides of the present invention are shown to have increased thermal fatigue resistance as compared to conventional carbides.

In another embodiment, tungsten carbide inserts, having a coarse (large) grain size, i.e., an average grain size larger than approximately 4 um as determined by the ASTM E-112 method, having improved fracture toughness and wear resistance were formulated. Preferably, the insert has a fracture toughness of at least 18 ksi (in)<sup>0.5</sup> when measured by the ASTM B-771 method. Additionally, the insert has a wear number of at least 2 when measured by the ASTM B-611 method. More preferably, the insert also has a hardness range of about 85.0 to about 87.0 Rockwell "A" hardness (Ra). In order to achieve the above fracture toughness and wear resistance, the cobalt content and the grain size of the carbide should be carefully selected.

In one embodiment, fracture toughness and wear resistance of an insert having a cobalt content of about 10% and a carbide relative particle size of about 9 were determined. The average carbide particle size as measured by ASTM E-112 method is approximately 5.8 um. This composition, termed "**910**", exhibited a fracture toughness of about 19 ksi (in)<sup>0.5</sup> (as measured in accordance with the ASTM B-771 method) and a wear number of about 2.3 (as measured in accordance with the ASTM B-611 method).

In one embodiment, fracture toughness and wear resistance of an insert having a cobalt content of about 12% and a carbide relative particle size of about 10 (assigned by determining the hardness) were determined. This composition, termed "**1012**", exhibited a fracture toughness of about 21.5 ksi (in)<sup>0.5</sup> (as measured in accordance with the ASTM B-771 method) and a wear number of about 2.2 (as measured in accordance with the ASTM B-611 method).

FIG. 7 shows conventional carbides (indicated by the composition numbers **411**, **510**, **512**, **614**, and **616**) as circles, while compositions in accordance with the present invention are shown as squares, diamonds, and triangles. The conventional carbides vindicated by the composition numbers **411**, **510**, **512**, **614**, and **616** generally follow an inverse relationship between fracture toughness and wear resistance, as indicated by curve 1 in FIG. 7. In contrast, embodiments of the present invention show that both increased fracture toughness and increased wear resistance can be achieved by controlling particle grain size and by using coarse grain carbide.

Control over particle size and cobalt content, therefore, provides a way to control the toughness and wear resistance of a particular insert. Accordingly, drill bits may be designed so that inserts having desired properties are selectively positioned on a roller cone. In some embodiments, it may be desirable to position inserts having different toughness and wear resistance properties on different rows. For example, in some embodiments, inserts positioned on interior rows may have a higher toughness and/or wear resistance than inserts

positioned on gage rows. However, other inserts arrangements are within the scope of the invention, and these particular embodiments are not intended to be limiting. Inserts in accordance with the present invention may be used on both inner and/or gage rows.

The present invention, therefore, provides a tough, wear resistant insert for use in rock bits. As a result of this, bits made in accordance with the present invention last longer, meaning fewer trips to change the bit, reducing the amount of rig down time, which results in a significant cost saving. In general, these advantages are realized through selecting appropriate carbide grain size and cobalt content.

While specific compositions have been disclosed, it should be noted that the present invention is not limited to the specific compositions disclosed above. Rather, preferred embodiments of the present invention include inserts having a fracture toughness of at least 18 ksi (in)<sup>0.5</sup> and a wear number of at least 2.0. Moreover, particular embodiments have a Rockwell hardness of at least 85. Also, the present invention specifically relates to inserts having a relative particle size of at least 8. Also, embodiments of the present invention preferably use cobalt in an arrangement of about 6%-18%. More preferably, the present invention relates to compounds using cobalt in the 8%-16%.

It is expressly within the scope of the present invention that other embodiments will include inserts formed from superhard materials having a relative particle size of 10 or greater. Under the system explained above, compositions **1008** and **1010** (and other suitable compositions within the hardness range of 85 to 87) are expressly within the scope of the present invention (See FIG. 5).

Moreover, while reference has been made to tungsten carbide and cobalt containing materials, other transition metal carbides, transition metal nitrides, and other suitable superhard materials are specifically within the scope of the present invention.

Also, while certain embodiments have been described, one of ordinary skill in the art will recognize that the scope of the invention is not limited to the specific compositions described above, but rather encompasses a number of coarse grain carbides having the desired properties. For example, it is within the scope of the present invention that compositions having a hardness of 83 to 85 Ra, a fracture toughness of 20 ksi (in)<sup>0.5</sup> and a wear number of at least 1.5 may also be used as a substrate in a PDC insert.

While the invention has been described with respect to a limited number of embodiments, those skilled in the art, having benefit of this disclosure, will appreciate that other embodiments can be devised which do not depart from the scope of the invention as disclosed herein. Accordingly, the scope of the invention should be limited only by the attached claims.

What is claimed is:

1. A rock bit comprising:  
a bit body;  
at least one roller cone rotatably coupled to the bit body;  
and

a plurality of cutting elements disposed on the at least one roller cone, wherein at least one of the plurality of cutting elements has a fracture toughness of at least 19 ksi (in)<sup>0.5</sup> and a hardness in a range of about 85 to 87 Rockwell A.

2. The bit of claim 1, wherein the at least one cutting element is disposed in at least one of a gage row and inner row.

3. The bit of claim 1, wherein the at least one cutting element comprises tungsten carbide.

4. The bit of claim 3, wherein the at least one cutting element comprises at least about 6% to 18% by weight cobalt.

5. The bit of claim 4, wherein the at least one cutting element comprises at least about 8% to 16% by weight cobalt.

6. The bit of claim 1, wherein the fracture toughness is at least 20.

7. The bit of claim 1, wherein the insert has a wear number of at least about 2.

8. The bit of claim 7, wherein the wear number is at least 2.2.

9. An insert for a rock bit, the insert having a fracture toughness of at least about 19 ksi (in)<sup>0.5</sup> and a hardness in a range of about 85 to 87 Rockwell A.

10. An insert for a rock bit, comprising:

tungsten carbide particles; and  
a cobalt binder disposed around the particles, wherein a grain size of the tungsten carbide particles and a content of the cobalt binder are selected to provide a fracture toughness of at least about 19 ksi (in)<sup>0.5</sup> and a hardness in a range of about 85 to 87 Rockwell A.

11. The insert of claim 10, wherein the cobalt binder comprises at least about 6% to 18% by weight.

12. The insert of claim 11, wherein the cobalt binder at least about 8% to 16% by weight cobalt.

13. The insert of claim 10, the fracture toughness is at least 20.

14. The insert of claim 10, wherein the tungsten carbide particles have a relative particle size of at least 8.

15. The insert of claim 10, wherein the tungsten carbide particles have an average particle size of greater than 4 microns.